

## 1

3,573,915

PHOTOGRAPHIC SILVER HALIDE EMULSIONS  
CONTAINING NITRO-SUBSTITUTED OR UN-  
SUBSTITUTED CINNAMIC ACID OR CINNAMAL-  
DEHYDEGiacomo Luciani and Fritz Dersch, Binghamton, N.Y.,  
assignors to GAF Corporation, New York, N.Y.  
No Drawing. Filed Nov. 16, 1966, Ser. No. 594,675

Int. Cl. G03c 1/34, 1/06, 1/76

U.S. Cl. 96—67

10 Claims

## ABSTRACT OF THE DISCLOSURE

A light-sensitive silver halide material having thereon a light-sensitive silver halide emulsion layer and containing, in the light-sensitive silver halide layer or in a layer in contact therewith, as an antifogging and stabilizer a compound having the formula:



where R is either



and n is 1 or 2.

This invention relates in general to photography and in particular to the provision of novel antifogging and stabilizing compounds for use in connection with the preparation and/or processing of photographic silver halide emulsions.

It is well known that light-sensitive materials such as gelatin silver halide emulsion exhibit a marked tendency to fog. The term "fog" as used in the photographic art connotes that portion of the density obtained upon development which arises by virtue of factors other than the photographic exposure. The fog may be attributable to a number of influences including, for example, excessive ripening of the emulsion, prolonged storage of the film and especially under conditions of elevated temperature and/or humidity, as well as by prolonged development of the exposed emulsion, etc.

Resort to rapid-developing operations which usually require the use of elevated temperatures likewise presents severe problems of fog.

As is well known, it is conventional practice in the photographic art to incorporate into silver halide emulsions various types of sensitizing agents in order to enhance their sensitometric response. For example, gold or sulphur sensitizing agents or combinations of both have been extensively employed for such purposes. Invariably, however, prior attempts to achieve ultimate speed in photographic emulsions so sensitized have been to a large extent vitiated by the concomitant occurrence of fog.

Furthermore, similar fogging problems are encountered when employing sensitizers of the reduction type, such sensitizing agents usually being employed to augment the sensitizing properties of gold, sulphur and the like. As examples of compounds known to function as reduction sensitizers in silver halide emulsions there may be mentioned in particular the following: imina-amino-methane-sulfonates; hydrazine and hydrazine derivatives; certain amines such as diethylenetriamine, triethylenetetramine, triethanolamine, silene compounds having a silicon-hydrogen bond, spermine, sodium formaldehyde sulfoxolate, stannous chloride, alkali metal sulfite; sugars, such as lactose, dextrose, ascorbic acid and the like. However, like many of their predecessors, the use of the afore-

## 2

mentioned compounds has likewise been encumbered by severe fogging problems and especially when employed in the preparation of photographic silver halide emulsions of the high-speed type.

5 The foregoing problems have in many instances necessitated resort to the use of antifogging compounds such as benzotriazole, nitro-benzimidazole, phenylmercapto-tetrazole and the like. However, these particular compounds have been ascertained to provide somewhat sub-optimum results since, while serving as effective antifogging agents, they display a pronounced tendency to reduce emulsion speed. To a great extent, the depression on emulsion sensitivity has more than offset any possible benefits arising from their use.

15 Considerable investigation likewise indicates that the gelatin itself may be a source of fogging problems. Quite obviously, the use of gelatins which are not properly balanced with regard to their content of sensitizing, restraining and antifogging substances frustrates attempts

20 to alleviate the fogging problem. Despite the fact that the manufacturers of photographic gelatins are, for the most part, highly skilled in controlling the proper content of sensitizers, antifogging agents, etc., e.g., by careful selection and treatment of raw materials, bones and hides, as well

25 as the careful control of the acid or alkaline treatment of the extraction of gelatin, and selection of filter aids, it is nevertheless frequently experienced that the gelatin material remains a causal factor with regard to fog. While the substantial majority of commercial gelatins have been ascertained to be offensive in this regard, the fogging problem has been found to be highly manifest with pig-skin, chicken feet and rabbit skin type gelatins and especially when utilized in the preparation of emulsions of the ammonia type.

30 35 Photographic silver halide emulsions are usually provided with one or more speed-increasing agents, e.g., the polyoxyalkylenes and derivatives thereof for purposes of compensating for the depression in sensitometric response caused by the antifogging agent. However, the net result has often been a re-establishment of the fogging problem.

The fogging problem is also aggravated by the use of hardening agents for the photographic emulsion, e.g., formaldehyde, glyoxal, etc.

40 45 In accordance with the discovery forming the basis of the present invention, it has been found that the antifogging and stabilization characteristics of light-sensitive silver halide emulsions can be synergistically modified to advantage by the utilization of a particular class of chemical compounds in connection with the preparation and/or processing of such emulsions.

50 55 Thus, a primary object of the present invention resides in the provision of improved antifogging and stabilizer compounds in which the foregoing and related disadvantages are eliminated or at least mitigated to a substantial degree.

Another object of the present invention resides in the provision of light-sensitive silver halide emulsions containing a compound which stabilizes the emulsion against fogging while exhibiting little, if any, tendency to reduce the speed or contrast of such emulsions.

60 65 A further object of the present invention resides in the provision of light-sensitive silver halide emulsions and photographic elements prepared therewith containing an antifogging compound which is substantially devoid of any tendency to reduce the sensitivity of the emulsion to light of longer wave length due to the presence of one or more sensitizing dyes.

A still further object of the present invention resides 70 in the provision of a process for the treatment of an exposed photographic silver halide emulsion wherein at least one of the steps of pretreating or developing the

emulsion is effected in the presence of a novel stabilizing compound to be more fully described hereinafter.

The attainment of the foregoing and related objects is made possible in accordance with the broader aspects of the present invention by the incorporation in a light-sensitive photographic element of, developing solution and/or pretreatment solution of a compound of the following structural formula:



wherein R is selected from the group consisting of



and wherein n represents 1 or 2.

The compounds included by the above depicted structural formula may be summarized as follows:



o-Nitrocinnamaldehyde



m-Nitrocinnamaldehyde



p-Nitrocinnamaldehyde



o-Nitrocinnamic acid



p-Nitrocinnamic acid



m-Nitrocinnamic acid



cinnamic aldehyde



cinnamic acid

The novel stabilizer compounds of the present invention can be prepared according to well known techniques. For example, the preparation of the nitro-cinnamic acids is described in Bellstein, vol. 9, pp. 604-606; the preparation of the nitro cinnamaldehydes is described in Organic Synthesis, vol. 33, p. 60.

Improved fog reduction and other beneficial effects are obtained when the aforementioned compounds are incorporated into the silver halide emulsion as "ripening finals" or as "coating finals." As is well known, ripening finals are added during the ripening or sensitivity increasing stage of the emulsion making process. Such additions may be effected before, during or after the decomposition of the soluble silver salt such as silver nitrate by means of a soluble halide such as potassium bromide, sodium chloride or the like in the presence of a suitable colloid carrier such as gelatin, polyvinyl alcohol, solubilized casein albumen or the like.

Coating finals are added to the emulsion just prior to coating on a suitable support such as glass, paper or film at the time when the emulsion has nearly attained its maximum sensitivity.

It will also be understood that the novel stabilizers of the present invention may be incorporated in a layer adjacent to the sensitized layer such as an anti-abrasion layer. The stabilizing compound may be utilized in concentrations varying over a relatively wide range; for example, when added to the light sensitive silver halide emulsion layer as a ripening final, it is found that optimum realization of results provided herein are assured with stabilizer concentrations ranging from as low as 25 milligrams up to about 500 milligrams per 1 mole of silver halide. The concentration selected within the aforesaid range will depend to a large extent on the type of emulsion employed and thus, it is advisable to determine the optimum concentration from case to case. If added during the emulsion preparation state, stabilizer concentrations ranging from 2 to 500 milligrams per 1 mole of silver halide are found to be quite suitable.

The stabilizer compounds contemplated herein can be applied in a variety of ways to impart stability to photographic elements. As previously mentioned, they may be included as a constituent of the emulsion layer, of a surface layer over the emulsion or alternatively, over the base or support.

Further embodiments of the present invention contemplate the addition of such compounds to at least one of the developing, fixing, washing, drying, etc., solutions utilized in the processing of the exposed emulsion.

In general, it is found that the improvements provided by the present invention are particularly manifest according to procedures whereby development is effected in the presence of said stabilizer compounds. This, of course, would be the case should the stabilizer be included in the light-sensitive photographic element, the developing solution and/or suitable developer pre-bath. In any event, when incorporated into the photographic developer or other processing bath, the stabilizers of the present invention are preferably employed in concentrations ranging from about 10 to about 500 milligrams per liter of solution, with a range of about 20 milligrams to about 200 milligrams per liter being particularly preferred.

In addition to being useful in orthochromatic and panchromatic emulsions, the stabilizers may also be used in nonsensitized emulsions, X-ray emulsions, paper emulsions, color emulsions and the like. If used with sensitizing dyes, they may be added to the emulsion before or after dye addition. Moreover, the present stabilizers may also be employed in conjunction with other known anti-fogging and stabilizers, reduction or sulfur sensitizers, metal and noble metal sensitizers or in combination with other additive agents and the like.

The stabilizer may also be employed in gelatin or other water-permeable colloids including polyamides or a mixture of gelatin with a polyamide as described in U.S.

Patent No. 2,289,775; polyvinyl alcohol and gelling compound as described in U.S. Patent No. 2,249,537; polyvinyl acetaldehyde acetal resins and partially hydrolyzed acetate resins described in U.S. Patent Nos. 1,939,422 and 2,036,092; cellulose derivatives, e.g., cellulose nitrate, cellulose acetate, and the lower fatty acid esters of cellulose including sample and mixed esters and ethers of cellulose and the like.

When preparing the photographic emulsion in accordance with the present invention, a solution of the stabilizer in a suitable solvent, such as water, alcohol, dimethyl formamide, N-methyl-2-pyrrolidone, or alcohol-water mixture adjusted to a neutral or slightly alkaline pH, i.e., about 6 to 8 is made up and the solution mixed with the emulsion at any convenient stage during its preparation, but preferably during ripening or just prior to coating.

The following examples are given for purposes of illustrating the present invention in greater detail, and are not to be considered in any way as being limitative thereof.

#### EXAMPLE I

A high speed negative ammonia emulsion was prepared using the formula described on page 332, Photographic Chemistry, vol. 1, by Pierre Glafkides (1958). A pigskin gelatin was used. This emulsion was called (a). A second emulsion (b) was prepared which differed from emulsion (a) in that we used, in the second ripening (after washing) 1 cc. of a 5% solution of o-nitrocinnamaldehyde in N-methyl-2-pyrrolidone.

Those emulsions were then readied for coating on film base, that is, melted at 40° C., necessary coating finals were added, such as stabilizers and hardeners. Emulsion samples were coated on a suitable cellulose ester base and dried. Samples of these film coatings were then exposed in a Type IB Sensitometer and developed in a developer of the following composition:

|                                | Grams |
|--------------------------------|-------|
| Metol                          | 1.5   |
| Sodium sulfite, anhydrous      | 45    |
| Sodium bisulfite               | 1     |
| Hydroquinone                   | 3     |
| Sodium carbonate, monohydrated | 6     |
| Potassium bromide              | 0.8   |
| Water to make 1 liter.         |       |

The sensitometric results were as follows:

|           | Relative speed | Fog 12' developer |
|-----------|----------------|-------------------|
| Emulsion: |                |                   |
| (a)-----  | 100            | .25               |
| (b)-----  | 100            | .12               |

#### EXAMPLE II

Example II differs from Example I in that the pigskin gelatin was replaced with an inert bone gelatin. There was added to the second ripening (after washing), a gold thiocyanate solution, which was prepared according to Glafkides (see Example I), page 319. There was also added a solution 1:10,000 of Na<sub>2</sub>S<sub>2</sub>O<sub>3</sub> as a sulfur sensitizer (Glafkides, p. 284) and a solution of hydrazine as a reduction sensitizer. The pH and pAg was adjusted by adding dilute sulfuric acid and KBr solution. Since the optimum amounts of these solutions depend on the selection of the gelatin, they have to be determined from case to case by fractional experiments (see Statistical Methods for Chemists by W. J. Youden, 1951, pp. 106-115). The so-prepared emulsion is called (a). Emulsion (b) differed from emulsion (a) in that we used 2 cc. of a 5% solution of p-nitrocinnamic acid in the after ripening per 1 kg. emulsion. The results were:

|           | Relative speed | Fog 12' developer |
|-----------|----------------|-------------------|
| Emulsion: |                |                   |
| (a)-----  | 100            | .26               |
| (b)-----  | 100            | .11               |

#### EXAMPLE III

Example III differs from Example II in that p-nitrocinnamic acid was replaced by m-nitrocinnamic acid.

#### EXAMPLE IV

Example IV was conducted similarly to Example II. However, the reduction sensitizer hydrazine was replaced by a solution 1:10,000 of stannous chloride, while in emulsion (b) the p-nitrocinnamic acid was replaced with o-nitrocinnamaldehyde.

#### EXAMPLE V

Example I was repeated except that the pigskin gelatin employed in emulsion sample (b) received a pre-treatment as follows:

To 1 liter of a 10% solution of pigskin gelatin at 40° C. there were added 24 cc. of a 5% solution of o-nitrocinnamaldehyde. After this addition, the so-prepared gelatin solution is chilled and dried and ground. The results were:

|           | Relative speed | Fog 12' developer |
|-----------|----------------|-------------------|
| Emulsion: |                |                   |
| (a)-----  | 100            | .28               |
| (b)-----  | 100            | .12               |

#### EXAMPLE VI

Example VI is similar to Example II; however, the Na<sub>2</sub>S<sub>2</sub>O<sub>3</sub> employed in emulsion sample (a) was replaced by thioacetamide. 1 cc. thioacetamide 1:10,000 can take the place of 20 cc. Na<sub>2</sub>S<sub>2</sub>O<sub>3</sub> 1:10,000. Emulsion sample (b) is like (a) but contains in addition, o-nitrocinnamaldehyde. The results are similar to those in Example II.

#### EXAMPLE VII

Example VII is similar to Example VI, but, instead of thioacetamide, diethyldithiocarbamic acid was used with almost identical results.

#### EXAMPLE VIII

A photographic silver halide emulsion as described in Example II was readied for coating on a suitable base, finals were added, such as stabilizers, coating aids, e.g., certain surfactants and as a hardener was added glyoxal in amounts of 40 cc. (5% solution) per 0.6 mole silver halide. This emulsion is called (a). A similar emulsion (b) but containing 10 cc. of a 1/2% solution of o-nitrocinnamaldehyde was also coated. The results were as follows:

|           | Relative speed | Fog 12' developer |
|-----------|----------------|-------------------|
| Emulsion: |                |                   |
| (a)-----  | 100            | .25               |
| (b)-----  | 100            | .12               |

#### EXAMPLE IX

A high speed negative ammonia emulsion was prepared using the formula described on p. 332, Photographic Chemistry, vol. 1 by Pierre Glafkides (1958). A pigskin gelatin was used. This emulsion was called (a). A second emulsion (b) was prepared which differed from emulsion (a) in that there was used, in the second ripening (after washing) 2 cc. of a 5% solution of cinnamaldehyde in ethanol. These emulsions were then readied for coating on film base, that is melted at 40° C., necessary coating finals were added, such as stabilizers and hardeners. Emulsion samples were coated on a suitable cellulose ester base and dried. Samples of these film coatings were then

exposed in a Type IB Sensitometer and developed in a developer of the following composition:

|                                | Grams |
|--------------------------------|-------|
| Metol                          | 1.5   |
| Sodium sulfite, anhydrous      | 45    |
| Sodium bisulfite               | 1     |
| Hydroquinone                   | 3     |
| Sodium carbonate, monohydrated | 6     |
| Potassium bromide              | 0.8   |
| Water to make 1 liter.         |       |

The sensitometric results were as follows:

|           | Relative speed | Fog 12' developer |
|-----------|----------------|-------------------|
| Emulsion: |                |                   |
| (a)-----  | 100            | .25               |
| (b)-----  | 100            | .14               |

#### EXAMPLE X

Example X differs from Example IX in that the pigskin gelatin was replaced with an inert bone gelatin. To the second ripening (after washing) was added a gold thiocyanate solution, which was prepared according to Glafkides (see Example I) p. 319. There was also added a solution 1:10,000 of  $\text{Na}_2\text{S}_2\text{O}_3$  as a sulfur sensitizer (Glafkides p. 284) and a solution of hydrazine as a reduction sensitizer. The pH and  $\text{pAg}$  was adjusted by adding dilute sulfuric acid and  $\text{KBr}$  solution. The so-prepared emulsion is called (a). Emulsion (b) differed from emulsion (a) in that there was used 2 cc. of a 5% solution of cinnamaldehyde in the after ripening per 1 kg. emulsion. The results were:

|           | Relative speed | Fog 12' developer |
|-----------|----------------|-------------------|
| Emulsion: |                |                   |
| (a)-----  | 100            | .26               |
| (b)-----  | 100            | .13               |

#### EXAMPLE XI

Example XI was conducted similarly to Example X. However, the reduction sensitizer hydrazine was replaced by a solution 1:10,000 of stannous chloride.

#### EXAMPLE XII

Example XII was conducted similarly to Example X with the exception of using in place of the hydrazine solution 1:10,000 a 5% solution of sodium sulfite. The results were almost identical to those in Example X.

#### EXAMPLE XIII

Example XII is repeated with the following exceptions: Emulsion sample (b) differed from emulsion sample (a) in that it contained in the second ripening, 1 gram of a polyethylene glycol of an average molecular weight of 4,000. Emulsion sample (c) differed from emulsion sample (b) in that it contained in addition, 2 cc. of a 5% solution of benzaldehyde.

#### EXAMPLE XIV

Example I is repeated except that the pigskin gelatin employed in the preparation of emulsion sample (b) is subjected to the following pre-treatment:

To 1 liter of a 10% solution of pigskin gelatin at 40° C. there was added 24 cc. of a 5% solution of cinnamaldehyde. After this addition, the so-prepared gelatin solution is chilled and dried and ground. The results were:

|           | Relative speed | Fog 12' developer |
|-----------|----------------|-------------------|
| Emulsion: |                |                   |
| (a)-----  | 100            | .28               |
| (b)-----  | 100            | .16               |

#### 8 EXAMPLE XV

Example XV is similar to Example II; however, the  $\text{Na}_2\text{S}_2\text{O}_3$  employed in emulsion sample (a) was replaced with thioacetamide. 1 cc. thioacetamide 1:10,000 can take the place of 20 cc.  $\text{Na}_2\text{S}_2\text{O}_3$  1:10,000. Sample (b) is like (a) but contains in addition, cinnamaldehyde. The results are like those in Example II.

#### EXAMPLE XVI

10 Example XVI is similar to Example XV, but instead of thioacetamide, diethyldithiocarbamic acid was used with almost identical results.

#### EXAMPLE XVII

15 Example XVII is like Example XIII except that the polyethylene glycol was replaced by 10 cc. of a 1% solution of diethylene triamine.

#### EXAMPLE XVIII

20 Example XVIII is like Example XVII except that the diethylene triamine was replaced by triethanol amine.

#### EXAMPLE XIX

25 The photographic silver halide emulsion described in Example II, was readied for coating on a suitable base, finals were added, such as stabilizers, coating aids, e.g., certain surfactants and as a hardener was added glyoxal in the amount of 40 cc. of a 5% solution per 0.6 mole silver halide. This emulsion is called (a). A similar emulsion (b) was coated but there was added 10 cc. of a 1/2% solution of cinnamaldehyde. The results were as follows:

|           | Relative speed | Fog 12' developer |
|-----------|----------------|-------------------|
| Emulsion: |                |                   |
| (a)-----  | 100            | .25               |
| (b)-----  | 100            | .15               |

#### EXAMPLE XX

40 Example XX is similar to Example XIX. However, formaldehyde was used in place of glyoxal. The results were almost identical to those described in Example XIX.

45 The present invention has been disclosed with respect to certain preferred embodiments thereof, and there will become obvious to persons skilled in the art various modifications, equivalents or variations thereof which are intended to be included within the spirit and scope of this invention.

What is claimed is:

50 1. A light-sensitive silver halide emulsion containing as an antifogging and stabilizer a compound of the following structural formula:



55 wherein R is selected from the group consisting of



60 and wherein n represents 1 or 2.

65 2. A light-sensitive silver halide emulsion according to claim 1 wherein said antifogging and stabilizer compound comprises o-nitrocinnamaldehyde.

3. A light-sensitive silver halide emulsion according to claim 1 wherein said antifogging and stabilizer compound comprises p-nitrocinnamic acid.

70 4. A light-sensitive silver halide emulsion according to claim 1 wherein said antifogging and stabilizer compound comprises m-nitrocinnamic acid.

75 5. A light-sensitive silver halide emulsion according to claim 1 wherein said antifogging and stabilizer compound comprises o-nitrocinnamic acid.

6. A light-sensitive silver halide emulsion according to claim 1 wherein said antifoggant and stabilizer compound comprises m-nitrocinnamaldehyde.

7. A light-sensitive silver halide emulsion according to claim 1 wherein said antifoggant and stabilizer compound comprises p-nitrocinnamaldehyde.

8. A light-sensitive silver halide emulsion according to claim 1 wherein said antifoggant and stabilizer compound comprises cinnamaldehyde.

9. A light-sensitive silver halide emulsion according to claim 1 wherein said antifoggant and stabilizer compound comprises cinnamic acid.

10. A light-sensitive photographic element comprising a base and a light-sensitive silver halide emulsion, said light-sensitive silver halide emulsion containing as an antifoggant and stabilizer a compound of the following structural formula:



wherein R is selected from the group consisting of



5 and



10 and wherein n represents 1 or 2.

#### References Cited

Chem. Absts., vol. 57, 335b.

15 NORMAN G. TORCHIN, Primary Examiner

M. F. KELLEY, Assistant Examiner

U.S. Cl. X.R.

20 96-95, 66.5, 109